

## UNITED STATES PATENT OFFICE

2,160,881

## LUBRICANT

Clarence M. Loane and Bernard H. Shoemaker,  
Hammond, Ind., assignors to Standard Oil  
Company, Chicago, Ill., a corporation of Indiana

No Drawing. Application June 10, 1937,  
Serial No. 147,483

## 20 Claims.

(Cl. 87—9)

This invention relates to lubricants and, in particular, to addition agents imparting to lubricants improved properties.

Our invention has particular utility in preventing and/or inhibiting the corrosion of "hard metal" alloy bearings such as copper-lead, cadmium-nickel, and cadmium-silver bearings which, to a large extent, have replaced soft metal bearings such as Babbitt metal in the trend toward internal combustion engines having high compression ratios and having increased acceleration and increased speed characteristics. The use of the "hard metal" bearings has created lubricating and corrosion problems, particularly in connection with "highly refined" oils, some of which may be very corrosive to the "hard metal" bearings.

By "highly refined" lubricating oils we mean viscous oils which have a minimum viscosity in the range of S. A. E. 10 oils and which have been subjected to such refining processes such as, for example, solvent extraction, that the paraffinicity of the oil is markedly increased. It has been found that highly refined lubricating oils cause corrosion to alloy bearings of the cadmium-silver type to the extent of 5 mg./cm.<sup>2</sup> and even greater when such bearings are submerged for 25 hours or less in an air agitated oil which has been pre-oxidized at about 340° F. for 25 to 50 hours. The motor oils may be highly refined lubricating oils as such or mixtures of highly refined lubricating oils with less highly refined lubricating oils, or stated in another way, mixtures of corrosive oils and non-corrosive oils, examples of the latter being lubricating oil fractions from Winkler crude or crudes of the Winkler type.

We have found that corrosion to hard metal alloy bearings of the cadmium-silver type by highly refined mineral lubricating oils can be inhibited by adding to such oils a small amount, up to 2% but preferably 0.25% to 0.75% of an organic ester of selenic acid selected from the group consisting of selenic acid esters having the general formula



Y

in which R is a radical selected from the group consisting of alkyl, chloralkyl, aryl, chloraryl, hydro aryl and aralkyl, X is an element selected from the group consisting of oxygen and sulfur and Y is a halogen.

Specific examples of compounds within the above classes are: dibutyl selenate, diethyl selenate, diphenyl selenate, didodecyl selenate, di-lauryl selenate, dicyclohexyl selenate, chlorbutyl

chloroselenate, phenyl chloroselenate, butyl phenyl selenate, phenyl propyl selenate, dodecyl chloroselenate, propyl chloroselenate, dichlorbutyl selenate, dibutyl thioselenate, diphenyl thioselenate, chlorphenyl chloroselenate.

To determine the effectiveness of the organic esters of selenic acid in inhibiting corrosion to hard metal alloy bearings of the cadmium-silver type in the presence of corrosive mineral lubricating oils, the same are tested by submerging test strips of cadmium-silver alloy in an oil corrosive to such materials in the absence of an inhibitor, and another set of the same alloy test strips are submerged in the oil to which is added 0.25% of an inhibitor and the oils maintained at a temperature of about 341° F. while passing 10 liters of air per hour through the oils. The test strips are removed periodically and weighed and the time required for the strips to lose 5 mgs./sq. cm. of surface noted. With dibutyl selenate as the corrosion inhibitor the following results were obtained:

| Oil                                 | Time for 5 mgs.<br>loss per sq. cm.<br>of surface | 25 |
|-------------------------------------|---------------------------------------------------|----|
| Control.....                        | Less than 1 day.                                  | 30 |
| Control+0.25% dibutyl selenate..... | 4 to 5 days.                                      | 35 |

The above data clearly indicate the effectiveness of the organic esters of selenic acid in inhibiting corrosion to hard metal alloys of the cadmium-silver type in the presence of corrosive mineral lubricating oils.

We have also discovered that the hereinbefore described compounds effectively reduce engine wear.

While we have described our invention with a specific embodiment thereof, it is to be understood that the same is merely illustrative of the invention and not a limitation thereof, except insofar as the same is defined in the appended claims.

We claim:

1. A motor oil non-corrosive to hard metal alloy bearings having the corrosive susceptibility of alloys of the group consisting of cadmium-silver alloys, cadmium-nickel alloys and copper-lead alloys containing an organic ester of selenic acid selected from the group consisting of selenic acid esters having the general formula  $OSe(XR)_2$  and



Y

45

50

55

in which R is a radical selected from the group consisting of alkyl, aryl, hydro aryl, aralkyl, chloralkyl and chloraryl, Y is a halogen and X is an element selected from the group consisting of 5 oxygen and sulfur, said organic ester of selenic acid being added in an amount not greater than about 2% but sufficient to render said motor oil non-corrosive to said hard metal alloys.

2. A motor oil non-corrosive to hard metal alloy bearings having the corrosive susceptibility of alloys of the group consisting of cadmium-silver alloys, cadmium-nickel alloys and copper-lead alloys containing an organic ester of selenic acid having the general formula  $OSe(OR)_2$  in which 10 R is a radical selected from the group consisting of alkyl, aryl, hydro aryl, aralkyl, chloralkyl and chloraryl, said organic ester of selenic acid being added in an amount not greater than about 2% but sufficient to render said motor oil non-corrosive to said hard metal alloys.

3. A motor oil non-corrosive to hard metal alloy bearings having the corrosive susceptibility of alloys of the group consisting of cadmium-silver alloys, cadmium-nickel alloys and copper-lead alloys containing an organic ester of selenic acid having the general formula 15



30 in which R is a radical selected from the group consisting of alkyl, aryl, hydroaryl, aralkyl, chloralkyl and chloraryl and Y is a halogen, said organic ester of selenic acid being added in an amount not greater than about 2% but sufficient to render said motor oil non-corrosive to said hard metal alloys.

4. A motor oil non-corrosive to hard metal alloy bearings having the corrosive susceptibility of alloys of the group consisting of cadmium-silver alloys, cadmium-nickel alloys and copper-lead alloys containing not more than about 2% of a dialkyl selenate but in amounts sufficient to render said motor oil non-corrosive to said hard metal alloys.

45 5. A motor oil non-corrosive to hard metal alloy bearings having the corrosive susceptibility of alloys of the group consisting of cadmium-silver alloys, cadmium-nickel alloys and copper-lead alloys containing not more than about 2% of a diaryl selenate but in amounts sufficient to render said motor oil non-corrosive to said hard metal alloys.

55 6. A motor oil non-corrosive to hard metal alloy bearings having the corrosive susceptibility of alloys of the group consisting of cadmium-silver alloys, cadmium-nickel alloys and copper-lead alloys containing not more than about 2% of dibutyl selenate but in amounts sufficient to render said motor oil non-corrosive to said hard metal alloys.

60 7. A motor oil non-corrosive to hard metal alloy bearings having the corrosive susceptibility of alloys of the group consisting of cadmium-silver alloys, cadmium-nickel alloys and copper-lead alloys containing an organic ester of selenic acid having the general formula  $OSe(SR)_2$  in which R is a radical selected from the group consisting of alkyl, aryl, hydroaryl, aralkyl, chloralkyl and chloraryl, said organic ester of selenic acid being added in an amount not greater than about 2% but sufficient to render said motor oil non-corrosive to said hard metal alloys.

70 8. A mineral lubricating oil non-corrosive to hard metal alloy bearings having the corrosive susceptibility of alloys of the group consisting

of cadmium-silver, cadmium-nickel and copper-lead alloys which comprises a highly refined mineral lubricating oil normally corrosive to hard metal alloys and a small amount sufficient to render said highly refined mineral lubricating oil 5 non-corrosive to said hard metal alloys of an organic ester of selenic acid selected from the group consisting of selenic acid esters having the general formula  $OSe(XR)_2$  and selenic acid esters having the general formula 10



in which R is a radical selected from the group consisting of alkyl, aryl, hydroaryl, aralkyl, chloralkyl and chloraryl, Y is a halogen and X is an element selected from the group consisting of oxygen and sulfur. 15

9. A mineral lubricating oil non-corrosive to hard metal alloy bearings having the corrosive 20 susceptibility of alloys of the group consisting of cadmium-silver, cadmium-nickel and copper-lead alloys which comprises a highly refined mineral lubricating oil normally corrosive to hard metal alloys and a small amount sufficient to 25 render said highly refined mineral lubricating oil non-corrosive to said hard metal alloys of an organic ester of selenic acid having the general formula  $OSe(OR)_2$  in which R is a radical selected from the group consisting of alkyl, aryl, 30 hydroaryl, aralkyl, chloralkyl and chloraryl.

10. A mineral lubricating oil non-corrosive to hard metal alloy bearings having the corrosive susceptibility of alloys of the group consisting of cadmium-silver, cadmium-nickel and copper-35 lead alloys which comprises a highly refined lubricating oil normally corrosive to hard metal alloys and a small amount of sufficient to render said lubricating oil non-corrosive to said hard metal alloy of an organic ester of selenic acid 40 having the general formula.



in which R is a radical selected from the group 45 consisting of alkyl, aryl, hydroaryl, aralkyl, chloralkyl and chloraryl and Y is a halogen.

11. A mineral lubricating oil non-corrosive to hard metal alloy bearings having the corrosive susceptibility of alloys of the group consisting of cadmium-silver, cadmium-nickel and copper-lead alloys which comprises a highly refined lubricating oil normally corrosive to hard metal 50 alloys and a small amount sufficient to render said lubricating oil non-corrosive to said hard metal alloys of an organic ester of selenic acid having the general formula  $OSe(SR)_2$  in which R is a radical selected from the group consisting of alkyl, aryl, hydroaryl, aralkyl, chloralkyl and chloraryl. 55

12. A mineral lubricating oil non-corrosive to hard metal alloy bearings having the corrosive susceptibility of alloys of the group consisting of cadmium-silver, cadmium-nickel and copper-lead alloys comprising a highly refined lubricating oil normally corrosive to hard metal alloys 60 and a small amount sufficient to render said lubricating oil non-corrosive to said hard metal alloys of an alkyl selenate.

13. A mineral lubricating oil non-corrosive to 70 hard metal alloy bearings having the corrosive susceptibility of alloys of the group consisting of cadmium-silver, cadmium-nickel and copper-lead alloys comprising a highly refined lubricating oil normally corrosive to hard metal alloys 75

and a small amount sufficient to render said lubricating oil non-corrosive to said hard metal alloys of an aryl selenate.

14. A mineral lubricating oil non-corrosive to hard metal bearings having the corrosive susceptibility of alloys of the group consisting of cadmium-silver, cadmium-nickel and copper-lead alloys which comprises a highly refined mineral lubricating oil normally corrosive to hard metal alloys and a small amount of dibutyl selenate in sufficient quantity to render said lubricating oil non-corrosive to said hard metal alloys.

15. The method of lubricating hard metal alloy bearings having the corrosive susceptibility of alloys of the group consisting of cadmium-silver, cadmium-nickel and copper-lead alloys in internal combustion engines which comprises applying to said bearings a mineral lubricating oil comprising a highly refined petroleum lubricating oil normally corrosive to said bearings and a small amount sufficient to render said lubricating oil non-corrosive to said hard metal alloys of an organic ester of selenic acid selected from the group consisting of selenic acid esters having the general formula  $OSe(XR)_2$  and selenic acid esters having the general formula



30 in which R is a radical selected from the group consisting of alkyl, aryl, hydroaryl, aralkyl, chloralkyl and chloraryl, Y is a halogen, and X is an element selected from the group consisting of oxygen and sulfur.

35 16. The method of lubricating hard metal alloy bearings having the corrosive susceptibility of alloys of the group consisting of cadmium-silver, cadmium-nickel and copper-lead alloys in internal combustion engines which comprises applying to said bearings a mineral lubricating oil comprising a highly refined petroleum lubricating oil normally corrosive to said bearings and a small amount sufficient to render said lubricating oil non-corrosive to said hard metal alloys of an organic ester of selenic acid having the general formula  $OSe(OR)_2$  in which R is a radical selected from the group consisting of alkyl, aryl, hydroaryl, aralkyl, chloralkyl and chloraryl.

40 17. The method of lubricating hard metal al-

loy bearings having the corrosive susceptibility of alloys of the group consisting of cadmium-silver, cadmium-nickel and copper-lead alloys in internal combustion engines which comprises applying to said bearings a mineral lubricating oil comprising a highly refined petroleum lubricating oil normally corrosive to said bearings and an organic ester of selenic acid having the general formula



15 in which R is a radical selected from the group consisting of alkyl, aryl, hydroaryl, aralkyl, chloralkyl and chloraryl and Y is a halogen, said organic ester of selenic acid being added in a small but sufficient quantity to render said lubricating oil non-corrosive to said hard metal alloy.

20 18. The method of lubricating hard metal alloy bearings having the corrosive susceptibility of alloys of the group consisting of cadmium-silver, cadmium-nickel and copper-lead alloys in internal combustion engines which comprises applying to said bearings a lubricating oil comprising a highly refined petroleum lubricating oil normally corrosive to said bearings and 0.25% to 0.75% of an organic ester of selenic acid having the general formula  $OSe(SR)_2$  in which R is a radical selected from the group consisting of alkyl, aryl, hydroaryl, aralkyl, chloralkyl and chloraryl.

25 19. The method of lubricating hard metal alloy bearings having the corrosive susceptibility of alloys of the group consisting of cadmium-silver, cadmium-nickel and copper-lead alloys in internal combustion engines which comprises applying to said bearings a mineral lubricating oil comprising a highly refined petroleum lubricating oil normally corrosive to said bearings and from about 0.25% to about 3% of an alkyl selenate.

30 20. The method of lubricating hard metal alloy bearings having the corrosive susceptibility of alloys of the group consisting of cadmium-silver, cadmium-nickel and copper-lead alloys as described in claim 19 in which the alkyl selenate is dibutyl selenate.

CLARENCE M. LOANE.  
BERNARD H. SHOEMAKER.

## CERTIFICATE OF CORRECTION.

Patent No. 2,160,881.

June 6, 1939.

CLARENCE M. LOANE, ET AL.

It is hereby certified that error appears in the printed specification of the above numbered patent requiring correction as follows: Page 2, second column, line 38, claim 10, strike out the word "of"; page 3, second column, line 39, claim 19, for "3%" read 2%; and that the said Letters Patent should be read with this correction therein that the same may conform to the record of the case in the Patent Office.

Signed and sealed this 11th day of July, A.D. 1939.

Henry Van Arsdale

(Seal)

Acting Commissioner of Patents.